# EUROPEAN PATENT SPECIFICATION

(11) **EP 2 251 483 B1**
(45) Date of publication and mention of the grant of the patent: **31.10.2012**
(21) Application number: 10160132.6
(22) Date of filing: 16.04.2010
(51) Int. Cl.: D21H 19/10, D21H 19/24, D21H 19/48, D21H 19/62, D21H 25/16

(54) **High-printability coated paper and method for its production**
Beschichtes Papier mit einer höhen Bedruckbarkeit und Verfahren für seine Herstellung
Papier couché ayant une imprimabilité élevée et procédé pour sa fabrication

(30) Priority: 20.04.2009 IT VR20090054
(43) Date of publication of application: 17.11.2010
(73) Proprietor: FEDRIGONI S.P.A., 37135 Verona (IT)
(72) Inventor: Piano, Pierino, 38062, Arco TN (IT)
(74) Representative: Modiano, Micaela Nadia

(56) References cited:
- EP-A- 0 773 263
- EP-A1- 0 461 768
- US-A- 3 281 267
- US-A- 4 155 892
- US-A- 4 507 426
- US-A- 5 478 388
- US-A1- 2007 240 619

## Description

The present invention refers to a high-printability coated paper and to a method for its production.

Nowadays papers are known and widespread upon which special surface treatments are carried out, for example coatings that can confer special effects both in aesthetic and tactile terms.

Indeed, in the paper sector, new ideas and technical solutions are continually being sought that make it possible to obtain paper products that are innovative and special, and capable of attracting, intriguing and astonishing end users. As indicated above, one of the paths taken by paper makers is to develop new types of paper that have tactile properties which are different from the usual ones, while at the same time maintaining the normal characteristics of the paper substrate.

In particular it has been found that almost all paper products provided with surface finishings that provide the specific tactile sensations of "plastic effect" or "silk/leather effect" present substantially two types of drawback.

A first drawback is constituted by the extreme sensitivity of the coating layer to pressure, a phenomenon that leads to adhesiveness between successive coils of coated paper when it is spooled onto a roll or between successive sheets once the paper has been cut and stacked (in the jargon, this phenomenon is known as "blocking").

A second drawback is related to lower print quality on the above mentioned paper products compared to what can be obtained on traditional papers for graphic uses. Specifically, it has been found that there are difficulties in anchoring the ink, a lack of sharpness of the print typeset, and what is known as "setoff" owing to the ink slow drying speed.

US-4 507 426 discloses polymeric agents useful for thickening aqueous systems including latex paints and other aqueous coating compositions.

US 4 155 892 discloses a polyurethane thickener for aqueous compositions.

US 5 478 388 discloses a pigment for a coating composition for printing paper.

The aim of the present invention is to obtain a paper, and specifically a high-printability coated paper, that has a tactile sensation which is special and unique, different from other products present on the market.

Within this aim, an object of the present invention is to make available a high-printability coated paper that can be used for packaging and for printing using the methods normally used for natural or traditional coated papers, including for example offset, embossing, hot stamping, thermal imaging and silk-screen for printing, and cutting, punching, creasing, folding and gluing for packaging operations.

Another object of the invention is to provide a high-printability coated paper that, specifically, has a surface that is soft and smooth to the touch and which at the same time has an opacity such as to bring to mind the concept of softness, also in visual terms.

A further object of the invention is to make available a method for producing a new type of high-printability coated paper which is extremely reliable and efficacious.

A further object of the invention is to develop a high-printability coated paper that allows effective anchoring of the ink during printing and which, at the same time, is less subject to the phenomenon of blocking.

This aim, as well as these and other objects which will become better apparent hereinafter, are achieved by a high-printability coated paper, as defined in claim 1.

The invention also provides a method for producing coated paper, as defined in claim 4.

Further characteristics and advantages of the invention will become better apparent from the following detailed description of some preferred, but not exclusive, embodiments of a high-printability coated paper, and of its production method, according to the invention.

In the embodiments that follow, individual characteristics shown in relation to specific examples may in reality be interchanged with other, different characteristics, existing in other embodiments.

The present invention refers to a coated paper, particularly adapted to printing and packaging, which comprises a paper substrate that has at least one coated face.

According to the present invention, the coating comprises a layer, of substantially uniform thickness, of a composition that comprises a polyurethane-based polymeric material in a percentage comprised between 65% and 90% by weight of the total weight and latex in a percentage comprised between 5% and 20% by weight of the total weight.

In particular, such composition is constituted by an aqueous dispersion of polyurethane-based polymeric material and latex.

Advantageously, the composition also comprises talc in a percentage of less than 20% by weight of the total weight.

Advisably, the paper substrate has a grammage that is comprised between 85g/m² and 400 g/m², a Bendtsen roughness degree that is comprised between 50 ml/min and 200 ml/min and a water absorption index (Cobb index) that is comprised between 20 g/m² and 25 g/m².

Obviously, the paper substrates used can be white or mass-coloured.

More precisely, the polyurethane-based polymeric material comprises a film-forming bonding agent, which comprises dispersions of anionic urethane polymers having aliphatic rigid segments and flexible polyether and polyester segments.

In this regard, the use of the formula commercially known as "Rolflex 2090", which is made by Lamberti S.p.A. in Gallarate (Varese, Italy) and which comprises, as well as the abovementioned components, silica, formulation auxiliaries and functional additives, has been found to be particularly suitable.

Advantageously, the composition is applied to such at least one face of the paper substrate in a quantity comprised between 3 g/m² and 15 g/m², preferably between 5 g/m² and 10 g/m².

It has also been found to be particularly useful to ensure that the talc added to the composition has an average diameter of 2.0 microns and a granulometric distribution such that at least 45%, preferably at least 48%, of the particles have a diameter of less than 2 microns.

Advisably, the latex used is of the SBR (Styrene-Butadiene-Rubber) type, but obviously there is no reason why other types of latex such as, for example, acrylic-based latexes should not be used, even though experimental results for such latexes have not been shown to be as satisfactory.

Obviously it is possible to add coloured pigments to the composition, if desired, to give more intense colourings to the coated surface.

According to another aspect, the present invention provides a method for producing coated paper which provides for the deposition, by coating, on at least one face of a paper substrate, of a composition comprising a polyurethane-based polymeric material in a percentage comprised between 65% and 90% by weight of the total weight and latex in a percentage comprised between 5% and 20% by weight of the total weight.

Advisably, the composition comprises talc in a percentage of less than 20% by weight of the total weight.

By way of example, the coating comprises an air knife coating.

According to a particularly important aspect, the temperature of the ribbon of coated paper should be kept at a temperature lower than 30°C.

Specifically, the production method makes use of one or more spreading rollers to take the coating that has a composition comprising polyurethane-based polymeric material, latex and possibly talc, in the percentages indicated above from a containment receptacle and to transfer it onto a ribbon of paper substrate upon which the coating is to be executed.

The quantity of coating applied exceeds the desired end result and the operation to remove the excess quantity is carried out by means of a "calibrated air blast" or air knife located immediately downstream of the applicator rollers.

Subsequently there is a drying phase which takes place by means of various different technologies such as, for example, radiation drying using infrared rays, convection drying using hot-air hoods, or conduction drying using steam-heated cylinders.

This phase can be followed by an identical sequence of operations if it is desired to apply a coating to the other side of the paper substrate as well.

Lastly, any accessory operations (for example cooling, coating, smoothing) can be performed before spooling the paper in rolls.

It has been found by experimental analysis of the coated paper according to the invention that the tactile effect obtained is, in effect, extremely unusual and original and able to convey the concept of "softness", also in visual terms.

From tests carried out, it has also been verified that the "blocking" phenomenon is greatly reduced by the combined action of the latex. The optional addition of talc has also produced a degree of printability that is substantially similar to that of papers for graphic uses.

In addition, all the details can be replaced by other technically equivalent elements.

Where the technical features mentioned in any claim are followed by reference signs, those reference signs have been included for the sole purpose of increasing the intelligibility of the claims and accordingly, such reference signs do not have any limiting effect on the interpretation of each element identified by way of example by such reference signs.

## Claims

1. A high-printability coated paper, comprising a paper substrate that has at least one coated face, said coating comprises a layer of substantially uniform thickness of a composition comprising a polyurethane-based polymeric material in a percentage comprised between 65% and 90% by weight of the total weight and latex in a percentage comprised between 5% and 20% by weight of the total weight, the composition comprising talc in a percentage below 20% by weight of the total weight, said polyurethane-based polymeric material comprising a film-forming bonding agent, which comprises dispersions of anionic urethane polymers having aliphatic rigid segments and flexible polyether and polyester segments, said composition being applied on said at least one face in a quantity comprised between 3 g/m² and 15 g/m², preferably between 5 g/m² and 10 g/m², said talc having an average diameter of 2.0 microns and a particle size distribution such that at least 45% of the particles have a diameter of less than 2 microns.

2. The high-printability coated paper according to claim 1, **characterized in that** said paper substrate has a grammage comprised between 85 g/m² and 400 g/m².

3. The high-printability coated paper according to one or more of the preceding claims, **characterized in that** said latex is of the SBR (Styrene-Butadiene-Rubber) type.

4. A method for producing high-printability coated paper, **characterized in that** it comprises the step of depositing, by coating, on at least one face of a paper substrate, a composition comprising a polyurethane-based polymeric material in a percentage comprised between 65% and 90% by weight of the total weight and latex in a percentage comprised between 5% and 20% by weight of the total weight, the composition comprising talc in a percentage below 20% by weight of the total weight, said polyurethane-based polymeric material comprising a film-forming bonding agent, which comprises dispersions of anionic urethane polymers having aliphatic rigid segments and flexible polyether and polyester segments, said composition being applied on said at least one face in a quantity comprised between 3 g/m² and 15 g/m², preferably between 5 g/m² and 10 g/m² said talc having an average diameter of 2.0 microns and a particle size distribution such that at least 45% of the particles have a diameter of less than 2 microns..

5. The method according to claim 4, **characterized in that** said composition comprises talc in a percentage of less than 20% by weight of the total weight.

6. The method according to one or more of claims 4 and 5, **characterized in that** said coating comprises an air knife coating.

7. The method according to one or more of claims 4 and 5, **characterized in that** the temperature of the ribbon of coated paper is kept below 30°C.

## Patentansprüche

1. Beschichtetes Papier mit hoher Bedruckbarkeit, umfassend ein Papiersubstrat, das wenigstens eine beschichtete Seite aufweist, wobei die Beschichtung eine im Wesentlichen gleichmäfsig dicke Schicht einer Zusammensetzung umfasst, die ein Polymermaterial auf Polyurethanbasis in einem Prozentanteil zwischen 65 und 90 Gewichts-% des Gesamtgewichts und Latex in einem Prozentanteil zwischen 5 und 20 Gewichts-% des Gesamtgewichts enthält, wobei die Zusammensetzung Talkum in einem Prozentanteil von weniger als 20 Gewichts-% des Gesamtgewichts enthält, wobei das Polymermaterial auf Polyurethanbasis ein filmbildendes Haftmittel umfasst, das Dispersionen von anionischen Urethanpolymeren mit aliphatischen starren Segmenten und flexiblen Polyether- und Polyestersegmenten umfasst, wobei die Zusammensetzung auf wenigstens einer Seite in einer Menge zwischen 3 g/m² und 15 g/m², vorzugsweise zwischen 5 g/m² und 10 g/m² aufgebracht ist, wobei das Talkum einen mittleren Durchmesser von 2,0 Mikrometern und eine solche Partikelgrößenverteilung aufweist, dass wenigstens 45% der Partikel einen Durchmesser von weniger als 2 Mikrometern aufweisen.

2. Beschichtetes Papier mit hoher Bedruckbarkeit nach Anspruch 1, **dadurch gekennzeichnet, dass** das Papiersubstrat eine Grammatur zwischen 85 g/m² und 400 g/m² aufweist.

3. Beschichtetes Papier mit hoher Bedruckbarkeit nach einem oder mehreren der vorhergehenden Ansprüche, **dadurch gekennzeichnet dass** der Latex vom Typ SBR (Styrol-Butadien-Kautschuk) ist.

4. Verfahren zur Herstellung von beschichtetem Papier mit hoher Bedruckbarkeit, **dadurch gekennzeichnet, dass** es den Schritt umfasst, dass auf wenigstens einer Seite eines Papiersubstrats durch Beschichten eine Zusammensetzung aufgebracht wird, die ein Polymermaterial auf Polyurethanbasis in einem Prozentanteil zwischen 65 und 90 Gewichts-% des Gesamtgewichts und Latex in einem Prozentanteil zwischen 5 und 20 Gewichts-% des Gesamtgewichts enthält, wobei die Zusammensetzung Talkum in einem Prozentanteil von weniger als 20 Gewichts-% des Gesamtgewichts enthält, wobei das Polymermaterial auf Polyurethanbasis ein filmbildendes Haftmittel umfasst, das Dispersionen von anionischen Urethanpolymeren mit aliphatischen starren Segmenten und flexiblen Polyether- und Polyestersegmenten umfasst, wobei die Zusammensetzung auf wenigstens eine Seite in einer Menge zwischen 3 g/m² und 15 g/m², vorzugsweise zwischen 5 g/m² und 10 g/m² aufgebracht wird, wobei das Talkum einen mittleren Durchmesser von 2,0 Mikrometern und eine solche Partikelgrößenverteilung aufweist, dass wenigstens 45% der Partikel einen Durchmesser von weniger als 2 Mikrometern aufweisen.

5. Verfahren nach Anspruch 4, **dadurch gekennzeichnet, dass** die Zusammensetzung Talkum in einem Prozentanteil von weniger als 20 Gewichts-% des Gesamtgewichts enthält.

6. Verfahren nach einem oder mehreren der Ansprüche 4 und 5, **dadurch gekennzeichnet, dass** die Beschichtung eine Luftmesserbeschichtung umfasst.

7. Verfahren nach einem oder mehreren der Ansprüche 4 und 5, **dadurch gekennzeichnet, dass** die Temperatur des Bandes von beschichtetem Papier unter 30°C gehalten wird.

## Revendications

1. Papier couché ayant une grande imprimabilité, comprenant un substrat de papier qui a au moins une face revêtue, ledit revêtement comprenant une couche d'épaisseur pratiquement uniforme d'une composition comprenant un matériau polymère à base de polyuréthane en un pourcentage compris entre 65 % et 90 % en poids du poids total et du latex en un pourcentage compris entre 5 % et 20 % en poids du poids total, la composition comprenant du talc en un pourcentage inférieur à 20 % en poids du poids total, ledit matériau polymère à base de polyuréthane comprenant un agent de collage filmogène, qui comprend des dispersions de polymères d'uréthane anioniques ayant des segments rigides aliphatiques et des segments polyéther et polyester flexibles, ladite composition étant appliquée sur ladite au moins une face en une quantité comprise entre 3 g/m² et 15 g/m², de préférence entre 5 g/m² et 10 g/m², ledit talc ayant un diamètre moyen de 2,0 micromètres et une distribution de granulométrie telle qu'au moins 45 % des particules aient un diamètre inférieur à 2 micromètres.

2. Papier couché ayant une grande imprimabilité selon la revendication 1, **caractérisé en ce que** ledit substrat de papier a un grammage compris entre 85 g/m² et 400 g/m².

3. Papier couché ayant une grande imprimabilité selon une ou plusieurs des revendications précédentes, **caractérisé en ce que** ledit latex est du type SBR (caoutchouc de styrène-butadiène).

4. Procédé pour produire un papier couché ayant une grande imprimabilité, **caractérisé en ce qu'**il comprend l'étape consistant à déposer, par revêtement, sur au moins une face d'un substrat de papier, une composition comprenant un matériau polymère à base de polyuréthane en un pourcentage compris entre 65 % et 90 % en poids du poids total et du latex en un pourcentage compris entre 5 % et 20 % en poids du poids total, la composition comprenant du talc en un pourcentage inférieur à 20 % en poids du poids total, ledit matériau polymère à base de polyuréthane comprenant un agent de collage filmogène, qui comprend des dispersions de polymères d'uréthane anioniques ayant des segments rigides aliphatiques et des segments polyéther et polyester flexibles, ladite composition étant appliquée sur ladite au moins une face en une quantité comprise entre 3 g/m² et 15 g/m², de préférence entre 5 g/m² et 10 g/m², ledit talc ayant un diamètre moyen de 2,0 micromètres et une distribution de granulométrie telle qu'au moins 45 % des particules aient un diamètre inférieur à 2 micromètres.

5. Procédé selon la revendication 4, **caractérisé en ce que** ladite composition comprend du talc en un pourcentage inférieur à 20 % % en poids du poids total.

6. Procédé selon une ou plusieurs des revendications 4 et 5, **caractérisé en ce que** ledit revêtement comprend un revêtement à la lame d'air.

7. Procédé selon une ou plusieurs des revendications 4 et 5, **caractérisé en ce que** la température du ruban de papier couché est maintenue inférieure à 30°C.
